# EUROPEAN PATENT SPECIFICATION

(11) **EP 0 233 689 B1**
(45) Date of publication and mention of the grant of the patent: **11.07.1990**
(21) Application number: 87300244.8
(22) Date of filing: 12.01.1987
(51) Int. Cl.: C11D 3/12, C11D 3/22, C01B 33/34

(54) **Aqueous zeolite dispersion**
Wässrige Zeolithdispersion
Dispersion aqueuse de zéolithe

(30) Priority: 17.01.1986 JP 7328/86
(43) Date of publication of application: 26.08.1987
(73) Proprietor: LION CORPORATION, Sumida-ku Tokyo (JP)
(72) Inventor: Abe, Seiji, Yotsukaido-shi Chiba (JP); Nakamura, Masayoshi, Chiba-shi Chiba (JP)
(74) Representative: Lightfoot, Robert Oscar

(56) References cited:
- EP-A- 0 154 291
- FR-A- 2 512 690
- FR-A- 2 523 950

## Description

The present invention relates to a stable aqueous zeolite dispersion.

It is well-known in the art that zeolites have an excellent ion exchange capability, adsorption capability, and other capabilities and, therefore, are industrially utilised as, for example, a detergent builder. Zeolites are generally produced in the form of an aqueous dispersion by a hydrothermal reaction, and are often handled as an aqueous dispersion from the viewpoints of transportation and handling. For example, granulated detergents for garments (e.g. clothes and fabrics) are produced by first preparing a detergent slurry, followed by spray drying. However, since it is difficult uniformly to disperse fine powdery zeolites in an aqueous detergent slurry, preferably an aqueous zeolite dispersion is prepared before mixing with a detergent slurry.

An aqueous zeolite dispersion, however, is unstable because of the difference in the specific gravities of water and the zeolite. Therefore, the zeolite separates and settles in the aqueous dispersion when the aqueous dispersion is stored.

Various attempts have been made to stabilise the aqueous zeolite dispersion as can be seen with reference to the following patents Nos: FR-A 2 523 950, FR-A 2 512 690, EP-A 0 154 291, JP-A 5 191 898 and JP-A 54 155 200 .

For example, Japanese Unexamined Patent Publication (Kokai) No. 51-91898 proposes that alkyl phosphate esters, slightly water-soluble nonionic surfactants, and sulfonate anionic surfactants be added to the aqueous zeolite dispersions, and Japanese Unexamined Patent Publication (Kokai) No. 54-155200 proposes that water-soluble nonionic surfactants and compatible salts (e.g., inorganic sodium salts) be combined and added to the aqueous zeolite dispersions. However, these proposals still do not satisfy the stability requirements for a long term storage of the aqueous dispersion, or provide satisfactory handling properties.

Accordingly, the present invention seeks to eliminate the above-mentioned disadvantages of the prior art and to provide an aqueous zeolite dispersion having an excellent fluidity and good storage stability.

In accordance with the present invention, there is provided an aqueous zeolite dispersion comprising 40% to 55% by weight, in terms of anhydride, of fine zeolite and 0.001% to 0.1% by weight of a lipopolysaccharide produced by a microorganism belonging to sp. Acineto bactor ATCC No. 31012.

The zeolites usable in the present invention include natural and synthetic zeolites. Examples of the synthetic zeolites are type-A, type-X and type-Y. Of these zeolites, the use of type-A zeolite is preferable from the builder standpoint. The average particle size of the zeolite is preferably 0.1 to 10 gm, more preferably 0.5 to 5 wm, and the zeolite is formulated into the aqueous dispersion at a content of 40% to 55% by weight, preferably 44% to 50% by weight. A zeolite content of less than 40% by weight is not economically preferable. For example, since the solid content of a conventional detergent slurry is generally 35 to 40% by weight, the water content in the detergent slurry is increased, when an aqueous zeolite dispersion having a low solid concentration is added, and therefore, the spray drying load is undesirably increased. When the zeolite content is more than 55% by weight, it is difficult to treat the aqueous dispersion.

The lipopolysaccharides prepared from microorganisms belonging to sp. Acineto bactor are so-called biosurfactants, which are available from, for example, Petroferm (U.S.A.) under the Registered Trade Mark EMULSAN. "Emulsan" is an extracellular microbiological protein associated with lipopolysaccharides, which is produced by a microorganism belonging to sp. Acineto bactor (deposited as ATCC No. 31012).

Examples of such lipopolysaccharides are a-Emulsans (i.e., Neoemulsans), which are produced when mainly ethanol is used as a carbon source, and p-Emulsans (i.e., Protoemulsans), which are obtained when mainly crude oil or hexadecane is used as a carbon source. The preparation of these lipopolysaccharides and their use are described in EP-B 0 016 546.

According to the present invention, the lipopolysaccharides produced by a microorganism belonging to sp. Acineto bactor ATCC No. 31012 are formulated into the aqueous zeolite dispersion in an amount or 0.001% to 0.1% by weight, preferably 0.005% to 0.06% by weight. When the content of the lipopolysaccharide is less than 0.001% by weight, the stability of the resultant zeolite dispersion is reduced. On the other hand, when the content of the lipopolysaccharide is more than 0.1% by weight, handling of the resultant aqueous zeolite dispersion becomes difficult because the viscosity of the dispersion is increased and the fluidity thereof is reduced.

The aqueous zeolite dispersion according to the present invention may optionally contain any conventional optional detergent ingredients (e.g., anionic surfactant, sodium sulfate, sodium carbonate, sodium citrate, sodium silicate) unless the stability of the dispersion is adversely affected.

According to the present invention, the aqueous zeolite dispersion having a high fluidity even at a low temperature and an excellent storage stability, can be advantageously obtained by adding thereto the lipopolysaccharides produced by a microorganism belonging to sp. Acineto bactor.

### Examples

The present invention will now be further illustrated by, but is by no means limited to, the following Examples, wherein all parts and percentages are expressed on a weight basis unless otherwise noted. Aqueous zeolite dispersions (i.e., sample Nos. 1 to 5 in Table 1) having the following formulations were prepared.

The viscosity of the resultant aqueous zeolite dispersion was determined and the settling stability of the resultant aqueous zeolite dispersion was evaluated after storage, by a stability test.

The results are shown in Table 1.

The viscosity and the storage stability were determined as follows:
(1) Viscosity
The viscosity was determined at 20 r.p.m. at a temperature of 25_{°}C by using a B-type viscometer (i.e., a Brookfield type viscometer).
(2) Settling stability

A sample dispersion was taken in a glass bottle. The bottle was sealed and was allowed to stand at a temperature of 25°C. Thus, the stability after one day was determined. The upper clear transparency layer in the bottle was visually evaluated, and the lower settled gel product was determined in terms or % by volume, as follows. That is, a glass plate having a diameter of 5 mm was gently and vertically placed in the lower settled gel product layer from the top of the glass bottle. When the glass plate came to the settled gel product, the length of the glass plate was determined. The volume percentage based on the total volume was calculated from the length of the glass plate.

The storage stability was good when the volume percentage of the upper layer was 30% by volume or less, and when the volume percentage of the lower layer was 1% or less after storage for 9 days.

The results shown in Table 1 were evaluated in terms of the number of days for which the dispersion was maintained.

## Claims

1. An aqueous zeolite dispersion characterised by comprising 40% to 55% by weight, in terms of anhydride, of fine zeolite and 0.001% to 0.1% by weight of a lipopolysaccharide produced by a microorganism belonging to sp. Acineto bactor ATCC NO. 31012.

2. An aqueous zeolite dispersion as claimed in claim 1, wherein a content of the zeolite is 44% to 50% by weight.

3. An aqueous zeolite dispersion as claimed in claim 1 or claim 2, wherein a content of the lipopolysaccharide is 0.005% to 0.06% by weight.

4. An aqueous zeolite dispersion as claimed in any one of the preceding claims, wherein an average particle size of the zeolite is 0.1 to 10 wm.

5. An aqueous zeolite dispersion as claimed in any one of the preceding claims, wherein the lipopolysaccharide is a lipopolysaccharide produced by a microorganism belonging to sp. Acineto bactor ATCC No. 31012 using ethanol, crude oil or hexadecane as the major source of carbon.

## Patentansprüche

1. Wäßrige Zeolithdispersion, gekennzeichnet durch einen 40-55 gew.-%igen Gehalt (ausgedrückt als Anhydrid) Feinzeolith und einen 0,001-0,1 gew.-%igen Gehalt an einem Lipopolysaccharid, das durch einen zur Art Acineto bactor ATCC Nr. 31012 gehörenden Mikroorganismus produziert wurde.

2. Wäßrige Zeolithdispersion nach Anspruch 1, dadurch gekennzeichnet, daß der Zeolithgehalt 44-50 Gew.-% beträgt.

3. Wäßrige Zeolithdispersion nach Anspruch 1 oder 2, dadurch gekennzeichnet, daß der Gehalt an dem Lipopolysaccharid 0,005-0,06 Gew.-% beträgt.

4. Wäßrige Zeolithdispersion nach einem der vorhergehenden Ansprüche, dadurch gekennzeichnet, daß die durchschnittliche Teilchengröße des Zeoliths 0,1-10 µm beträgt.

5. Wäßrige Zeolithdispersion nach einem der vorhergehenden Ansprüche, dadurch gekennzeichnet, daß es sich bei dem Lipopolysaccharid um ein solches handelt, das durch einen zur Art Acineto bactor ATCC Nr. 31012 gehörenden Mikroorganismus unter Verwendung von Ethanol, Rohöl oder Hexadecan als Hauptkohlenstoffquelle produziert wurde.

## Revendications

1. Dispersion aqueuse de zéolite caractérisée en ce qu'elle comprend sur une base anhydre 40 à 55% en poids d'une zéolite fine et 0,001 à 0,1% en poids d'une lipopolysaccharide produit par un microorganisme appartenant à l'espèce Acineto bactor ATCC N° 31012.

2. Dispersion aqueuse de zéolite selon la revendicationi, dans laquelle la teneur en zéolite est de 44 à 50% en poids.

3. Dispersion aqueuse de zéolite selon la revendication 1 ou 2, dans laquelle la teneur en lipopolysaccharide est de 0,005 à 0,1% en poids.

4. Dispersion aqueuse de zéolite selon l'une quelconque des revendications précédentes, dans laquelle la taille moyenne des particules de zéolite est 0,1 à 10 µm.

5. Dispersions aqueuse de zéolite selon l'une quelconque des revendications précédentes, dans laquelle le lipopolysaccharide est un lipopolysaccharide produit par un microorganisme appartenant à l'espèce Acineto bactor ATCC n° 31012 utilisant l'éthanol, le pétrole brut ou l'hexadecane comme source principale de carbone.
